

Nov. 8, 1938.

H. R. DICKINSON

2,136,282

PROCESS OF TREATING WAXES

Filed July 25, 1935



Inventor

HENRY RANDEL DICKINSON

By

*Frank S. Hodges*

Attorney

## UNITED STATES PATENT OFFICE

2,136,282

## PROCESS OF TREATING WAXES

Henry Randel Dickinson, Grand Rapids, Mich.

Application July 25, 1935, Serial No. 33,148

9 Claims. (Cl. 196—17)

This invention is a process for imparting amorphous characteristics to normally crystalline waxes.

One of the objects of the invention is to so unite and commingle crystalline wax with an amorphous material, as to provide a homogeneous mass possessing marked amorphous characteristics. A further object is to regulate the homogenizing process in such manner as to control the hardness, plasticity and/or melting point of homogenized waxes.

The invention will be hereinafter fully set forth and particularly pointed out in the claims.

In the accompanying drawing, the figure is a diagrammatic view illustrating an apparatus for carrying out the invention, with parts shown in section.

In carrying out the invention, amorphous and crystalline waxes are mixed together, and the mixture subjected to high pressure by fluid or mechanical means, while in a state of fusion. The pressure employed is relatively high, preferably ranging from 10 pounds per square inch to 10,000 pounds per square inch. By means of this process, crystalline waxes may be made to simulate waxes which possess amorphous characteristics, and a wax of low melting point can be re-formed in such manner as to have a melting point which is much higher. By varying the amount of pressure, the hardness of the wax is materially increased and is highly useful for the purpose of rendering paper transparent. In addition to the foregoing, the plasticity of the wax so blended and treated with pressure is materially increased or changed.

Referring to the drawing, 10 indicates a melting tank which communicates with an autoclave 11 of standard type, by means of a pipe 12, controlled by a suitable valve 13. A second melting kettle or supply tank 14 is also connected with the autoclave 11 by means of a pipe 15, controlled by a valve 16. The autoclave 11 may be of any suitable or desired structure provided with the usual steam heating jacket 17, and with an internal agitator 18, which may be rotated in suitable manner (not shown). The heating temperature of the steam jacket is controlled by means of a temperature control device diagrammatically indicated at 19, and controlling a shut-off valve 20 in the steam-supply line, in accordance with variations of temperature within the autoclave. Connected with the autoclave 11 below the liquid level, by means of a pipe 21 is an air or fluid pump or compressor 22, of any desired construction.

Leading from the bottom of the autoclave is an outlet pipe 23, to which is connected a pipe 24, which discharges into the inner passage of a nozzle N having an outer air pressure passage 31 controlled by valve 32, and leading to the atmosphere, which discharges into an expansion chamber 25. The chamber 25 is also provided with a drain connection 26, controlled by a valve 27, the outlet pipe 23 being controlled by a valve 28. The expansion chamber 25 is connected with 10 a suitable collection tank 29 by means of a pipe 30, as shown.

In operation, a crystalline wax such as paraffin, is melted within the kettle 10, and the amorphous material, such as ozocerite wax, asphalt, 15 or the like, is melted within the tank 14. When the two materials reach the desired melted state, the respective valves 13 and 16 are opened, and the two materials, while in the melted state, flow into the autoclave 11, through the respective 20 pipes 12 and 15, being intimately mixed and commingled by means of the agitator 18, in an obvious manner. It is to be understood, of course, that the steam jacket of the autoclave maintains the molten condition of the mixed 25 materials. During the agitation step, compressed air or other pressure fluid is pumped or supplied into the autoclave by the compressor 22, whereby the melted mixture within the autoclave is permeated with air and subjected to a very high 30 degree of pressure, preferably ranging from 10 pounds per square inch to 10,000 pounds per square inch, according to the results desired. In other words, the higher the pressure, the more complete the process. After the mixing and 35 pressure steps have been completed, the materials will have become intermingled and homogenized into an amorphous mass permeated with air, and may then be drawn off from the autoclave through the pipes 23 and 24 into the 40 expansion chamber 25. The sudden reduction of pressure as the mixture is admitted to the expansion chamber results in a somewhat explosive action which produces the final complete dissemination of the mixture within itself. The 45 mass is collected in chamber 25, the air escapes through the line 30, and the mass is drawn off through pipe 26 and valve 27 into a suitable receptacle (not shown), in which the mass is allowed to cool and solidify. If it should be desired 50 to separate the mixture into fine particles, the valve 27 is closed and the valve 32 is opened, whereupon the pressure will cause the mixture to be discharged through pipe 24 into the expansion chamber 25 with sufficient velocity to 55

draw in air through the passage 31, thereby breaking the mixture up into extremely fine, hard particles, which are sufficiently cooled by the air drawn in to maintain their individuality.

5 After the pulverizing of the mixture, there is still sufficient pressure, or an exhauster may be used, to force the finely divided particles into a collection tank 29, where the material may be stored as long as desired.

10 It is to be understood that although paraffin wax, ozocerite wax and/or asphalt have been mentioned as examples of materials to be blended, the invention is not limited to these particular substances. For instance, non-solvent oils, liquids or fats of any suitable characteristics may be blended with either of the original waxes before being subjected to the stages of the process or in the process, and the entire mass, after processing, will be rendered amorphous and so completely homogenized that the oil, liquid or fat will resist separation from the waxes. By thus mixing oils, liquids or fats, amorphous waxes and crystalline waxes, full control may be had over the final product with respect to the characteristics of plasticity, hardness and reactions to heat and chemicals.

The advantages of the invention will be readily understood by those skilled in the art to which the invention belongs. For instance, by means 30 of the process above described, crystalline waxes are made to simulate amorphous waxes, and rendered capable of the same uses and fabrication treatments as amorphous waxes. Another advantage is that any desired hardness, plasticity 35 and/or reaction to heat and chemicals is obtainable. The use of this process will also render more amorphous, rubbery or flexible a mixture of crystalline wax with asphaltum or bitumen.

Having thus explained the nature of the invention and described an operative manner of constructing and using the same, although without attempting to set forth all of the forms in which it may be made, or all of the forms of its use, what is claimed is:—

45 1. The process of mixing crystalline wax and amorphous material comprising mechanically mixing melted crystalline wax and melted amorphous material within a closed chamber, and independently introducing a compressible fluid into said chamber during the mixing stage and maintaining said fluid under high pressure until the melted ingredients of the melted mixture are completely homogenized by the pressure of said fluid and assume distinctly amorphous characteristics.

50 2. The process of mixing crystalline wax and amorphous material comprising separately melting crystalline wax and the amorphous material, causing the melted materials to intermingle within a closed chamber while in their melted state and independently introducing a compressible fluid into said chamber during the mixing stage, said fluid being maintained under high pressure until the melted ingredients of the mixture are completely homogenized by the pressure of said fluid and assume distinctly amorphous characteristics.

55 3. The process of mixing crystalline wax and amorphous material comprising feeding a stream of crystalline wax and a separate stream of melted amorphous material to a closed container, maintaining said wax and amorphous material in a melted condition and mechanically mixing them within the container while in a molten state, and independently introducing a compress-

sible fluid into said closed chamber during the melting stage and maintaining said fluid under high pressure until the ingredients of the melted mixture are completely homogenized by the pressure of said fluid and assume distinctly amorphous characteristics.

4. The process of imparting amorphous characteristics to crystalline wax comprising mixing paraffin wax and ozocerite wax together while both waxes are in a melted state, subjecting the melted mixture within a closed chamber to the action of a compressible fluid maintained under high pressure within said chamber, and suddenly reducing the pressure upon the mixture.

5. The process of mixing crystalline wax and amorphous material comprising melting said crystalline wax and said amorphous material and commingling them within said closed chamber while in the melted state, and independently introducing a compressible fluid into said chamber during the melting stage, and maintaining said compressible fluid under high pressure within said chamber until the melted ingredients of the mixture are completely homogenized by the pressure of said fluid and assume distinctly amorphous characteristics, discharging the homogenized material from the closed chamber, and suddenly releasing the pressure thereon as the homogenized material is so discharged.

6. The process of mixing crystalline wax and amorphous material comprising melting said crystalline wax and said amorphous material and commingling them within said closed chamber while in the melted state, and independently introducing a compressible fluid into said chamber during the melting stage, and maintaining said compressible fluid under high pressure within said chamber until the melted ingredients of the mixture are completely homogenized by the pressure of said fluid and assume distinctly amorphous characteristics, and while said homogenized mixture is still in a melted state, discharging the same into a space which is normally maintained at a much lower pressure than the pressure in the first mentioned chamber.

7. The process of mixing crystalline wax and amorphous material comprising melting said crystalline wax and said amorphous material and commingling them within said closed chamber while in the melted state, and independently introducing a compressible fluid into said chamber during the melting stage, and maintaining said compressible fluid under high pressure within said chamber until the melted ingredients of the mixture are completely homogenized by the pressure of said fluid and assume distinctly amorphous characteristics, and atomizing the melted homogenized material at a temperature sufficiently low for the atomized particles to maintain individuality.

8. The process of mixing crystalline wax and amorphous material comprising mixing said wax and said amorphous material within a closed chamber while in a melted state, adding oil to the melted mixture while contained within said chamber, and independently introducing a compressible fluid into said chamber during the melting stage and maintaining said fluid under high pressure until the ingredients of the mixture are completely homogenized by the pressure of said fluid and assume distinctly amorphous characteristics, and suddenly reducing said pressure at the end of the mixing stage.

9. The process of mixing crystalline wax and amorphous material comprising melting said

5 crystalline wax and said amorphous material and commingling them within said closed chamber while in the melted state, and independently introducing a compressible fluid into said chamber during the melting stage, and maintaining said compressible fluid under high pressure within said chamber until the melted ingredients of the mixture are completely homogenized by the pressure of said fluid and assume distinctly

amorphous characteristics, withdrawing the homogenized material from the closed chamber while in a melted state and under said pressure, and pulverizing the withdrawn material by discharging it into a lower pressure atmosphere 5 while in a melted state and in such manner as to suddenly relieve the material of said high pressure.

HENRY RANDEL DICKINSON.